

Oct. 4, 1955

J. B. DIFFENDERFER

2,719,355

CARBONIZED METAL AND METHOD OF MAKING IT

Filed June 28, 1947

2 Sheets-Sheet 1

*Fig. 1*



*Fig. 2*



*Fig. 3*



*Fig. 4*



*Fig. 5*



*Fig. 6*



*Fig. 7*

INVENTOR  
John B. Diffenderfer  
EY  
William A. Zalesak  
ATTORNEY

Oct. 4, 1955

J. B. DIFFENDERFER

2,719,355

CARBONIZED METAL AND METHOD OF MAKING IT

Filed June 28, 1947

2 Sheets-Sheet 2



INVENTOR.

*John B. Diffenderfer*

BY

*William A. Zalesak*  
ATTORNEYS.

**1**

2,719,355

**CARBONIZED METAL AND METHOD OF  
MAKING IT**

John B. Diffenderfer, Catlin Township, Chemung County, N. Y., assignor to Radio Corporation of America, a corporation of Delaware

Continuation of abandoned application Serial No. 757,752, June 28, 1947. This application October 3, 1952, Serial No. 312,945

3 Claims. (Cl. 29—195)

My invention relates to carbon coated metal for use where good thermal emittance or heat radiating power is desirable as, for example, in evacuated devices, such as electric discharge devices where metal parts or elements radiate heat in vacuum during operation of the device. In electronic discharge devices like radio tubes such carbonized metal is particularly useful for tube elements, such as carbonized anodes or plates, for heat radiators attached to tube elements, such as grids, and for similar uses. My invention further relates to carbonized metal or plate material for electrodes for electric discharge devices, to methods of making such material, and to improved carbonized electrodes, such as plates or anodes, for use in thermionic discharge devices.

This is a continuation of my co-pending application Serial No. 757,752, filed June 28, 1947, for Carbonized Metal and Method of Making it, now abandoned, and assigned to the same assignee as said co-pending application.

In electronic discharge devices the metal parts, other than the electron emissive elements, are generally kept as cool as feasible. To this end, in thermionic discharge devices, such as radio tubes, these other or cold electrodes such as grids, plates, and other electrodes which receive or are subjected to the electron current during operation are blackened to increase their thermal emittance or heat radiating power, usually by a coating of some form of carbon. For reasons of economy in manufacture on a large scale, long strips of sheet electrode metal are usually carbonized by a continuous process and the electrodes then formed from the carbonized strip. Nickel has been used extensively as the metal for the electrodes. The ferrous metals, such as mild steel, iron, or iron alloys, are much cheaper than nickel and could be used if satisfactorily carbonized, but they could not be carbonized with satisfactory results. The conventional gas carbonizing method in which the metal is heated in a hydrocarbon atmosphere to a temperature at which the hydrocarbon decomposes and deposits carbon on the metal is not satisfactory when applied to ferrous metals. The temperature necessary to obtain from the hydrocarbon atmosphere the right kind of carbon is so high that there is some carburization or case hardening of the ferrous metal, which is objectionable for several practical reasons. Gas carbonizing hardens steel, even when the steel has a thin coat of nickel, and impairs the strength of the metal. As the electrodes must be made with great precision, die forming is difficult unless the carbonized strip is quite ductile and practically non-resilient. Any carburization of a ferrous metal strip decreases the ductility of the metal and hardens it so much that the wear on the dies which form the electrodes is excessive.

To obtain by commercially acceptable methods a firmly adherent coating of carbon on a metal surface is difficult, as apparently no real bonding of the carbon to the metal can be attained by heat treatment. Various expedients such as sand or steel blasting, etching, and

**2**

other methods have been used to roughen the surface of the metal in efforts to improve the adhesion of the carbon coating. Experience has shown that adhesion of the carbon coating to the metal and the thermal emittance of the carbon coated electrode is a function of and is dependent on the texture of the metal surface rather than on its roughness.

The principal object of my invention is to provide metal, such as plate or electrode material, with a surface of novel texture to which a coating, such as carbon, adheres more firmly than to the surfaces obtained by conventional methods, and which when coated with carbon, especially carbon wholly or partly in the form of colloidal graphite, has a thermal emittance or heat radiating power which is very considerably greater than that of the best commercially used carbonized material of the conventional kind and closely approaches that of a black body.

Another object of the invention is to provide on an annealed ferrous metal such as mild steel a firmly adherent carbon coating so applied that the carbon does not affect or modify the properties of the metal in any way.

A further object of my invention is to provide a satisfactorily carbonized and commercially useful electrode of ferrous or other metal which may, if desired, be made to have a thermal emittance greater than 90% of that of a black body.

Another object of my invention is to provide electrode stock or material comprising a strip or sheet of ferrous or other metal which is practically dead soft, is easily shaped in dies into electrodes of precise dimensions, has a comparatively soft surface compressible in the forming dies, and preferably has a coat of carbon paint which is so firmly adherent that it will withstand the working of the material in the electrode forming dies.

Another object of the invention is to provide a simple, rapid and continuous process for treating a steel or similar metal strip to form on its surface a spongy porous layer or matrix of novel texture to which a coating, such as carbon, adheres very firmly and with which a carbon coating forms carbonized metal having thermal emissivity very close to that of a black body.

In accordance with my invention a base of sheet metal, preferably, but not necessarily, a ferrous metal such as mild steel, although some other metal, such as nickel, may be used, is surfaced by bonding to one or both of its surfaces a very firmly adherent porous layer or matrix bonded to the base and composed of fine metallic particles sintered to one another to leave voids forming fine pores. In the preferred embodiment the metallic particles are metal sponges which have microscopic pores and crevices, and which are sintered to one another and to the metal base to form a cohesive mass molecularly bonded to the base and having a novel texture and porosity or sponginess because of the porosity due to the minute pores or voids between the particles sintered to the base and to one another and also to the microscopic porosity of the individual particles or metal sponges. The matrix may be composed of particles which are nearly all about the same size, or it may be composed of a mixture of particles of different sizes. The surface of the matrix of the surfaced base is usually rough and irregular, with a multitude of minute pits and depressions, and also of microscopic pits on the surface of the porous sponges or particles of metal. The layer or matrix of small sintered porous particles or sponges of metal has a novel texture and structure and is preferred because it has been found to hold a coating, such as carbon, more firmly than the porous matrix composed of fine solid particles of metal sintered to one another and bonded to the metal base.

The fine metal particles of the matrix are best obtained by the controlled reduction in place on the base of fine particles of oxide of the metal constituting the particles. For example, to obtain the preferred form of matrix composed of porous particles, finely ground metallic oxide, preferably nickel oxide, is uniformly distributed over and in contact with the surface of the base as a layer of powdered oxide with the grains of the powder in contact with one another and held on the foundation base by a binder which disappears when moderately heated. The powdered oxide is reduced to metallic nickel by heating the metal strip with the layer of nickel oxide on it in a reducing atmosphere, such as hydrogen, preferably at about 800° C. to 1100° C., until the grains of nickel oxide are reduced without fusion to minute nickel sponges which have microscopic pores and crevices. The temperature at which the nickel oxide is reduced is high enough to form nickel sponges as the grains of powdered nickel oxide are reduced, but is too low to melt the reduced nickel into a solid mass. These individual porous nickel sponges effectively retain their individuality although they are sintered to one another and to the solid metal base. As a result, the metal foundation has a metallic nickel surface layer or matrix which is of novel texture, is soft, well bonded to the base strip, and porous because of minute voids between the metal sponges and also of the microscopic pores in the sponges. The metal base surfaced with my novel matrix constitutes a foundation which, when properly carbonized, produces a carbonized electrode superior to the conventional kind. A coating, such as carbon preferably consisting in large part of colloidal graphite, applied to and covering this matrix is found to be exceptionally adherent. The adhesion of the carbon particles to the matrix is greater than their cohesion to one another, hence the carbon coating cannot be removed as sheets or flakes, but only as carbon powder, the particles of which adhere very strongly to the foundation. Such a carbonized electrode retains the carbon coating unusually well and has a thermal emittance or heat radiating power which may be as high as 98% of that of a black body.

The foundation strip is preferably made by a continuous process in which the metal base strip, coated with a layer of powdered nickel oxide, is passed through a hydrogen furnace in which the oxide is reduced, preferably at such a temperature and under such conditions that the reduced metallic nickel forms porous particles or nickel sponges sintered to one another and bonded to the base, thus producing a foundation consisting of a sheet of metal surfaced with a layer or matrix of the desired texture and structure.

The carbon may be applied to the foundation in various ways, preferably as a kind of carbon paint consisting of very finely divided graphite, lampblack or other form of carbon suspended in a thin binder. The carbon paint may be applied in any convenient way, such as spraying, brushing, or dipping, but preferably by a continuous immersion or drag coating process in which the foundation with the novel porous matrix is in the form of a strip which is passed through a thin suspension of colloidal graphite in a vehicle such as alcohol, to which may be added some nitrocellulose or similar binder. Some very finely divided lampblack may be added if a very black coating is desired. The suspension is of such low viscosity as to be quickly absorbed by the porous matrix, such as ink is absorbed by blotting paper, and this impregnates the matrix with very finely divided carbon, and also cover the surface of the matrix with a coat of the carbon paint. The foundation is dried, leaving on it a thin coat of the carbon or graphite paint with a surface which usually has in general much the same contour as the rough and irregular surface of the matrix. When the vehicle of the carbon paint is driven off there is left on the foundation a carbon coating which is practically bonded to the metal.

My invention will be better understood from the following description in connection with the accompanying drawing in which merely for purposes of illustration there is shown one embodiment of my invention in a carbonized element, such as an anode or plate, of a thermionic tube, and my preferred method of making the anode or plate material from which the finished anode or plate is made, and in which:

Fig. 1 illustrates the surface of the porous matrix as seen in a photomicrograph with a magnification of 1000 diameters;

Fig. 2 illustrates the structure of the matrix as seen in a photomicrograph with a magnification of 1000 diameters in cross-section;

Fig. 3 illustrates on a greatly enlarged scale the surface of the matrix composed of metal sponges sintered to one another to leave voids and minute pores;

Fig. 4 illustrates on a greatly enlarged scale a cross-section of the matrix structure illustrated in Fig. 3;

Fig. 5 illustrates a portion of the base coated with nickel oxide as seen in cross-section in a photomicrograph;

Fig. 6 illustrates in cross-section the base with a matrix formed from the nickel oxide coating of Fig. 5 and seen as in a photomicrograph upon which is shown merely for illustration the carbon coating of the finished element;

Fig. 7 is a view of a carbonized plate part having two deep drawn projections and four right angle bends and made successfully on a large scale in accordance with my invention;

Fig. 8 is a fragmentary cross-section of the strip as it leaves the apparatus with a coat of carbon paint on it;

Fig. 9 shows in part schematically one example of the apparatus suitable for practicing my continuous process, and Fig. 10 a detail of the device.

One specific embodiment of my invention is in a carbonized plate or anode having, as indicated in the drawing, a metal foundation comprising a non-porous metal base 10, preferably a sheet of ferrous metal such as cold-rolled or mild steel about 5 mils thick, surfaced with a porous metallic matrix 11 consisting predominantly of nickel sponges or porous particles of nickel 12 having microscopic pores 13 and firmly and molecularly bonded to the base 10 and also sintered to one another. Photomicrographs show that the pores 13 are usually of an average size of about a tenth of a micron. The nickel sponges or porous particles of nickel retain in general their individuality, and are sintered to one another, with voids 14 between them forming minute capillary pores 15, many of which extend through the matrix to the base 10. These pores 15 are in general many times the size of the microscopic pores 13 of the nickel sponges, and may often be about the size of the nickel particles. I have found that I may apply to the matrix a carbon coating, preferably but not necessarily, so thin that the outer surface is in general of the same contour as the interface between the matrix and the carbon coating and therefore of the same general contour as the surface of the porous matrix 11, and achieve a carbonized electrode having thermal emittance or heat radiating power of from 90% to 98% that of a black body, with the carbon coating of such a character and so firmly adherent that there is practically no peeling, flaking off, or significant loss of carbon in use.

The microscopically porous nickel particles or nickel sponges 12 sintered to one another form a matrix of novel texture which is bonded to the base and has been found to bind a coating such as carbon more firmly to the metal base than has been achieved in previously known commercial practice by using surfaces roughened in conventional ways. The adherence of carbon to metal is not solely dependent on the degree or extent of roughness of the metal surface. The character of the roughness and the texture of the surface are much more important. Mechanical roughening of a metal surface by a single sand-

blasting or steel blasting deteriorates the metal and decreases its ductility by cold working and produces a surface only about one-half as rough as the surface of the matrix 11, and of a texture which does not bind the carbon to the metal nearly as well as the porous matrix 11. Blasting increases die wear because fine particles of the blasting material often adhere to the electrode metal. Repeated sand or steel blasting to increase the roughness of the surface deteriorates the metal still more, does not improve the texture for holding carbon, and is not feasible on account of cost and other objections. An oxidized strip of nickel or of nickel plated steel has only a very slightly roughened surface, which does not have the right texture to hold carbon as firmly as the matrix of my invention. Repeated oxidization and reduction of the nickel increases to some extent the roughness of the surface, but does not improve the texture for holding carbon, embrittles the nickel, and is not commercially feasible, largely on account of cost.

The matrix 11 of microscopically porous nickel sponges is most conveniently formed by applying to the base 10 a non-compacted layer of powdered nickel oxide in a binder, as indicated in Fig. 5, and reducing the nickel oxide under such conditions and at such temperature that the oxide is reduced without fusion to form the nickel sponges in place on the base and simultaneously molecularly bond them to the base and sinter them to one another with minute voids between them. The layer of nickel oxide may be formed on the base in various ways, preferably by means of a slurry or suspension of the powdered oxide in a binder and applied in various ways, as by brushing, spraying, or by immersing of the base in the suspension. A dry spray results in a matrix with a very rough surface, and a wet spray produces a smoother surface. The preferred way of applying the oxide is by the immersion or drag coating method, in which the base is coated by passing it through a bath of the suspension and then drying the coating. Commercial nickel oxide suitable for use in practicing my invention may be obtained on the market as a mixture of nickelous and nickelic oxides,  $\text{NiO}$  and  $\text{Ni}_2\text{O}_3$ , and is believed to be prepared from a natural ore by refining to eliminate sulphur and other impurities. The oxide is preferably ground by ball milling to a powder so fine that most of the grains are about 2 microns in diameter and less than 5% of the grains are larger than 5 microns, although a minor part of the powder may in some cases consist of much larger grains. A typical batch of nickel oxide powdered by ball-milling consisted of about 80% to 85% of grains or particles about 2 microns in diameter, 5% or more of particles between 2 microns and 5 microns, and the remainder of particles ranging in diameter from 5 or 6 microns up to 16 microns. These nickel oxide grains or particles 16 reduce to nickel sponges which usually are about the same size as the nickel oxide particles from which they are formed. These sintered sponges produce a matrix with a very uniform fine grained surface, best shown in Fig. 1, light grayish in color and about twice as rough as a single sand blasted nickel surface. It is obvious that a matrix with a rougher surface may be obtained by using larger grains of oxide. For immersion or drag coating the base with nickel oxide good results have been obtained with a slurry of the powdered nickel oxide suspended in an evanescent binder consisting of highly volatile butyl or amyl acetate and of some nitrocellulose. Suitable proportions are about 1500 grams of the nickel oxide powder to about 700 grams of amyl acetate and 35 grams of 40 second nitrocellulose. Some methanol, such as 250 grams, may be added to obtain the proper viscosity of the binder. This slurry coats the base evenly and when dried, leaves a suitable coat or layer of nickel oxide adhering to the base. I have found that good results are obtained when this binder has a viscosity of about 30 to 35 C. P. S. at 23° C., or with a

standard pipette of 145 to 170 seconds for 100 cc. of binder at 23° C.

The nickel oxide is preferably reduced by heating the oxide coated base, best shown in Fig. 5, in a reducing atmosphere, preferably hydrogen, at temperatures and for times ranging from about 800° C. for about ten minutes to 1100° C. for about one-half minute, which will ordinarily reduce the particles 16 of nickel oxide to nickel sponges 12. A desirable and convenient procedure is to heat to about 900° C. for about one minute. The preferred amount of reduced nickel constituting the matrix is about 5½ milligrams per square centimeter of the surface covered by the matrix, which produces a matrix about 1 mil thick on each side of the base. Good metal sponges form at about 900° C., which is below the transformation temperature of the mild steel of the base 11. Where the steel base is a mild steel strip, for example, about 5 mils thick, it may be passed through a reducing furnace of the conventional type about six feet long at a speed of about 8 feet per minute, the whole length of the tube being maintained at a temperature which heats the strip to the recommended temperature. Under these conditions the metal of the base, particularly if it is mild steel, is practically fully annealed and nearly dead soft, and usually has a negligible spring back, such as about 18 to 20 degrees, as compared with a spring back of about 50 to 60 degrees of gas carbonized nickel coated steel strip. The spring back test is well known, and one accepted test is described in a publication of the American Society of Testing Materials, test B-155.

Within a range of temperature of 800° C. to 1000° C. the nickel oxide is reduced without fusion to produce the nickel sponges which sinter to one another and are molecularly bound to the base by some nickel-iron alloy which forms at the interfaces of the nickel sponges and the steel base. At temperatures above the transformation point of most mild steels, which is about 930° C., some distortion of the steel strip and modification of the properties of the steel, such as ductility, may occur. At these higher temperatures the grains of nickel oxide may be reduced to solid metal particles, thus producing a matrix which is porous on account of voids between solid particles and holds a carbon coating quite well, but not as well as a matrix composed of nickel sponges. A matrix of solid particles may also be obtained by reducing the nickel oxide at a lower temperature, such as 750° C., for a much longer time, about one-half hour, which is usually not commercially feasible on account of cost. During the reduction there is some loss of volume in the layer of nickel oxide as it loses its oxygen and binder and the nickel particles sinter together resulting in the formation of a porous web-like matrix with minute pores and voids.

The matrix of sintered porous particles is rather soft and about 50% compressible, and contains no hard abrasive particles. Such a porous matrix of nickel can be deformed and burnished by a burnisher of copper, nickel, brass, or even of soft wood, and may be compressed to a considerable extent by the pressure of the plate forming dies, so that the die wear in shaping the foundation into electrodes is slight.

A metal base surfaced with a porous matrix in accordance with my invention and without a coating is a material useful for many purposes, especially in electronic discharge devices. As the material is well annealed and well degassed, it is suitable for wires and other elements of thermionic devices, and as it holds a coating very firmly, it is suitable for coated elements, such as carbon coated grids and if the base is nickel, for oxide coated filamentary cathodes and cathode sleeves.

The carbon coating 17 may be applied to the foundation in various known ways. The foundation with a nickel base 10 may be gas carbonized with good results. If the base 10 is a ferrous metal, such as mild steel or iron, either clear or with thin nickel plating, the carbon coating should be applied without subjecting the base to heat treat-

ment in the presence of carbon. Preferably, the carbon is applied by treating the matrix with a thin suspension or carbon slurry of very finely divided carbon, such as colloidal graphite in which as shown by photomicrographs, the particles range in size from about 1 micron to a small fraction much less than one-tenth of a micron; hence a large number of them are smaller than the microscopic pores 13 in the nickel sponges. I have achieved good results by immersion or drag coating the foundation with a kind of carbon paint consisting of a slurry of alcohol dag, which is a suspension of colloidal graphite in alcohol, and a small amount of a nitrocellulose binder which disappears when heated to moderate temperatures, such as 200° C. One illustrative example of a suitable carbon slurry is about 200 grams of alcohol dag, which is 160 grams methanol and 40 grams colloidal graphite, mixed with about 200 cc. of a medium drying binder consisting of about 1 part by weight of about equal parts of  $\frac{1}{2}$  second and 40 second nitrocellulose and about 12½ parts by weight of amy! acetate and diluted with about 250 cc. of butyl acetate and 200 cc. of methanol. The matrix has a degree and kind of porosity such that it absorbs the thin alcohol dag suspension much like blotting paper absorbs writing ink. With this slurry a carbonized electrode may be made with a grayish black carbon coating which is very effective. For a blacker carbon coating to give optimum heat radiation, a mixture of 100 grams of alcohol dag and 100 grams of lampblack may be used in place of the 200 grams of alcohol dag. The foundation is thoroughly wet with the slurry and dried, leaving as shown in Fig. 8 the foundation covered with a thin and very firmly adherent coat 18 of carbon paint composed of finely divided carbon and a small amount of binder.

The tube elements, such as plates, are made from the coated foundation, preferably by shaping them in dies in the usual way. The dried coat 18 of carbon paint is so adherent that it is not damaged in the dies, and in general no lubricant for the dies is necessary. Where the finished electrode is of complicated shape, such as shown in Fig. 7, having deep drawn portions and sharp bends, some lubrication of the dies may be advisable, in which case a lubricant such as machine oil which does not soften nitrocellulose may be used.

The coated element is finished and ready for use upon removal of the binder from the dried coat of carbon paint, preferably by heating in a neutral or non-oxidizing environment. The binder disappears upon heating to a moderate temperature, such as 200° C., leaving on the tube element a thin, firmly adherent carbon coating. This heating of the element may be done during exhaust of the tube in which it is mounted, but preferably is done prior to mounting the tube element in the electrode assembly.

In the preferred practice the shaped and coated elements are generally fired at about 800° C. in hydrogen for about ten minutes to prepare them for use. This firing first removes the binder from the dried coat of carbon paint and then also cleans and finishes the element. At this temperature and under these conditions there is negligible carburization or modification of the base by carbon. The result is a carbonized element, such as a plate, with a carbon coating of which the adhesion to the foundation is greater than its cohesion. Such a coating does not chip, peel, or flake off. If brushed, it may come off as powdered carbon, but not in the form of flakes or sheets, as often occurs with the conventional carbonized electrodes.

The carbon coating on the finished electrode is preferably as thin as feasible to produce a good black surface. For example, a successful coating has been found to weigh about 2 milligrams per square centimeter of surface of the foundation. While such a coating completely covers the matrix to an appreciable depth, it is very firmly bound to the base of the matrix and may be so thin that its surface has practically the same contour as the surface of the metallic matrix of the foundation. The carbon coating is so adherent that it cannot be scraped

from my carbonized anode mechanically without distorting the porous metal matrix. It can be removed without substantial alteration in the structure of the matrix by firing the carbonized anode at about 1100° C. for about ten minutes in hydrogen, such as line hydrogen, which contains some water vapor. In this way the substantially unaltered matrix 11 of the carbonized anode can be exposed.

Carbon coated anodes, for example, made as above described, have been found by comparative measurements to have much higher thermal emittance than similar conventional carbonized anodes. The thermal emittance of a carbonized anode embodying my invention is above 90% and usually about 95% to 98% of that of a black body, while the thermal emittance of similar conventional commercial carbonized anodes ranges from about 60% to somewhat less than 90% of that of a black body. These comparative measurements, made in air at 200° C. to avoid possible oxidation are valid up to the temperatures usually attained by the anodes during tube operation.

While I have described the preferred embodiment of my invention in which a sheet of mild steel is the base, the matrix is of metal sponges, and the carbon coating is a mixture of colloidal graphite and lampblack, it is to be understood that I may use other metals for the base or the matrix, provided the matrix metal particles may be reduced from the oxide in place on the face and will molecularly bond to the base and sinter to one another with capillary voids between them, and that other kinds of carbon coating may be used. For example, the base may be nickel or nickel plated iron, and iron oxide may replace a part of the nickel oxide where it is not deemed essential that all of the metal particles be of spongy structure.

My invention has marked commercial advantages, among them a marked reduction in cost. By only one heating in hydrogen, the matrix metal oxide is reduced in place and the reduced metal particles are sintered to one another and to the base, an inexpensive base metal such as iron or steel may be used, and the carbon coating can be applied more rapidly and at lower cost than by gas carbonizing; for example, largely because the peculiar porosity of the matrix enables it to absorb very quickly the carbon slurry, much as blotting paper absorbs ink, thus producing on the finished element a thin very adherent carbon coating which completely covers the matrix. Heretofore, iron could not be satisfactorily carbonized without a heat treatment in the presence of carbon with unavoidable resultant carburization and impairment of the metal. By my invention the iron is not impaired while being carbonized; and is in some respects improved by the degassing and annealing it undergoes during the reduction of the nickel oxide.

Among the structural and other features which distinguish a carbonized metal electrode embodying my invention from the carbonized metal electrode of the prior art are: a base of practically fully annealed metal which, if ferrous metal, such as mild steel, is practically dead soft and has a spring back of one-half or less of that of a gas carbonized nickel coated steel base, a porous metal matrix of novel texture on the base and comprising particles of metal sintered to one another and molecularly bonded to the base, and on the matrix an unusually adherent coating of carbon which does not peel or flake. This carbonized electrode has unusually high thermal emittance, which may be and usually is from 90% to 98% of that of a black body. The performance in thermionic tubes of my carbonized plates is so much better than that of the conventional carbonized plates that some desirable types of tubes which cannot be made with conventional carbonized plates can be made successfully with my carbonized plates and cannot be made commercially without them.

The preferred method of practicing my invention is a continuous process in which in general a steel strip is drag

or immersion coated with nickel oxide slurry, and the coated strip passed through a reducing furnace where the nickel oxide is reduced in place on the strip to form the matrix on the strip and thus produce the foundation which is then drag or immersion coated with the carbon paint or slurry to make the electrode stock or material from which tube elements, such as anodes may be quickly and economically made, preferably by shaping in dies.

This continuous process will be better understood from the following more detailed description in connection with the drawing, particularly Figs. 9 and 10. In this process the base 10, in the form of a strip of mild steel, such as is known commercially as No. 1010, and for convenience about 5 mils thick, is drawn off a supply reel 20, around pulley 23 and through an oxide slurry chamber 24 containing the nickel oxide slurry above recommended for drag coating. To apply the slurry in a thin, even coating, the strip 10 is passed around a pulley 25 in the chamber 24 and then out of the chamber and up through an applicator 26 which, as best shown in Fig. 10, may be a pipe with two diametrically opposite slots slightly larger than the strip 10 which passes through the slots with a slight clearance. The oxide slurry in the chamber 24 is continuously circulated through the pipe by pump 27 and overflows through both slots back into the chamber 24. To obtain an oxide coating that is uniform longitudinally of the strip, the oxide particles must be kept uniformly dispersed in the suspension by the pump, and the slurry maintained at constant viscosity, which may conveniently be done by adding from a tank 28 through a needle valve 29 a regulated quantity of methanol, or other volatile agent to the contents of the chamber 24.

The oxide slurry coated strip emerges from the applicator 26 and passes vertically into the vertical drying oven 30, which may be maintained at about 200° C. and in which the volatile constituents of the binder evaporate and thus keep the nickel oxide coating and the strip so cool that the nitrocellulose does not disappear. The strip, coated with a dried coat of nickel oxide slurry, passes from the drying oven into the vertical reducing furnace 31 through a bottom slot or opening slightly larger than the strip and providing only enough clearance to preclude scraping of the dried coating off the strip. The reducing furnace has an atmosphere of hydrogen or other reducing gas supplied through an inlet 31a at slightly above atmospheric pressure, and is run at a temperature which keeps the strip in the furnace at the chosen temperature within the range of 800° C. to 1100° C., thereby causing decomposition of the nitrocellulose and reduction of the nickel oxide. At the chosen temperature the nickel particles resulting from the reduction are well sintered to one another and molecularly bonded to the steel strip. The temperature of the strip in the furnace and its speed are such that while good adherence of the reduced nickel to the steel is achieved by incipient fusion of nickel iron alloy at the interface, the bulk of the reduced nickel is in the form of a porous matrix of microscopically porous nickel sponges. The furnace 31 is a usual type, about six feet long, and is maintained at about the same temperature from end to end. The strip may be passed through the furnace at a speed of about eight feet per minute. The cool strip entering the hot furnace at this speed is subjected to a rather great and sudden increase of temperature. This sharp temperature gradient is advantageous in producing the desired structure of the nickel matrix. A by-product of the reduction is water vapor which tends to have a decarburizing and softening action on the steel.

The strip 10 emerges from the furnace 31 as a foundation with a matrix coating of sintered metallic nickel which is soft, highly porous, and bonded to the metal strip. The extreme porosity can be readily shown by marking with ink, which is absorbed almost completely as by blotting paper. With the prior strips with which I am familiar, ink marks dry on the surface and remain

permanently visible as if on paper. Upon leaving the furnace the nickel surfaced strip passes through a cooling chamber 32, around pulley 33 enclosed in a gas tight housing, and down through another cooling chamber 34, from which it emerges through a bottom slot and at substantially room temperature. Both cooling chambers and the housing for the pulley 33 are kept filled with hydrogen from the furnace, as the cooling chamber 32 opens into the furnace and also into the housing around the pulley 33.

As the foundation strip emerges from the cooling chamber 34, it is ready for the application of a coating, such as carbon. It may be stored, if desired, and the coating applied later as a separate operation. I prefer to pass the foundation strip directly on down into a carbon applicator chamber 35, around pulley 36 in the chamber, and up through another applicator 37, similar to applicator 26, and through which flows the carbon slurry, maintained at proper viscosity by a small methanol tank 38 for supplying methanol through a needle valve 39, and circulated through the applicator 37 by a pump 40. The foundation strip, with a uniform coat of carbon paint or slurry which has entered the pores and crevices of the nickel matrix much as ink enters blotting paper, next enters drying oven 41, similar to the oven 30 and maintained at about 200° C. to produce a dried coat 18 of carbon paint on and covering the matrix. The binder in the carbon slurry binds the carbon particles together on the surface, in the pores, and in crevices of the nickel matrix. The carbon may be either amorphous or graphitic, depending upon the nature of the carbon added to the suspension in applicator chamber 35. The foundation strip with a dried coat of carbon paint 18, as shown in Fig. 8, passes out of the oven 41 and around pulley 42 to a reel, not shown, and then may be stored as electrode stock from which electrodes and tube elements may be made. The carbon can in this way be applied to the strip with the matrix surface much more rapidly than by gas carbonizing methods, in which the carbon is applied by deposition from hydrocarbon gases. A speed of eight feet per minute, which is ten times as rapid as the gas carbonizing process, has been obtained in my method.

With a 5 mil steel strip the coating of nickel matrix and carbon paint on both surfaces raises the thickness of the foundation strip at the most to only about 7.5 mils. No difficulty will therefore be encountered in making vacuum tube plates with dies designed for 5 mil strip, as the foundation strip made by my method with a coat of carbon paint on it is readily compressed in the dies. However, if desired, this foundation strip may be run through rolls and compressed. I have in this way reduced the coating on each surface of the strip to a thickness of less than 1 mil without materially affecting the heat radiating characteristics of the finished electrode. From metal coated by my improved method, compressed or not, carbonized electrodes may be made that have heat radiation power or thermal emittance more nearly approaching that of a black body than metal carbonized by any other method known to me.

An additional advantage of my method is that the steel strip as supplied by the manufacturer can be stored and then used without cleaning, as rust on the steel strip is reduced in the reducing chamber and oil film on the strip can also be tolerated.

The coat of carbon paint on the nickel matrix coated strip adheres very firmly to the nickel and does not pack in the dies when the tube parts are formed. The tube parts made therefrom may be fired in hydrogen at about 800° C. for 10 minutes, as customary, without depletion of the carbon. Another advantage of the electrode or plate stock made according to my invention is that the comparatively rigorous firing tends to degas and purify the material.

75 My method of carbon coating metal may be employed

with various metals. It will be found quite suitable for coating nickel strips as well as ferrous metal strips. It also can be used to obtain metal surfaces of two different metals sintered together and composed of metals that cannot be applied to each other by electrolytic plating or by any other method at all. For example, nickel and copper which will not co-deposit electrolytically are easily applied together. It is also possible to include non-metallic substances with the metals by mixing them in the slurry. Various other modifications may be made in the method and product without departing from the spirit of the invention.

What is claimed is:

1. A carbonized metal article comprising a sheet metal base, and a spongy rough surface bonding layer bonded to said base, said bonding layer having a coating thereon of colloidal graphite, said bonding layer consisting entirely of individually microscopically porous nickel particles sintered to one another, whereby empty spaces are provided in said bonding layer in the form of pores in the individual nickel particles and voids between the sintered nickel particles, the particles in contact with said base being sintered to the base for bonding said layer to the base; the outer surface of said bonding layer consisting of a layer of said particles, said particles in said layer defining voids therebetween and having pores therein communicating with said surface, said coating of colloidal graphite being in intimate contact with the surfaces of said particles in said layer defining said voids and the pores therein, whereby said coating is strongly adherent to said article to permit working of the article without loss of the coating and said coating is characterized by improved continuity on said outer surface for causing said article to have improved heat radiating properties.

2. A continuous method of making a metal strip having a coating of carbon thereon wherein the coating is characterized by improved adherence to assure freedom from loss during a subsequent working of the coated strips; said method comprising the steps of coating said metal strip with a non-compacted layer of finely powdered nickel oxide in a binder evanescent at a temperature below 900° C.; passing the coated strip through a furnace having a reducing atmosphere and a temperature of about 900° C. to reduce said nickel oxide to porous particles of nickel in situ on said strip, and to simultaneously

sinter said porous nickel particles to one another into a spongy layer and bond said layer to said strip, said temperature being below the temperature at which said porous particles collapse; passing said strip through a carbon slurry of very finely divided carbon suspended in a thin liquid binder, whereby said slurry is absorbed by said spongy layer and covers said spongy layer with a continuous coating of carbon, and drying said coating, whereby said coating is strongly adherent to said matrix and said coated metal strip is characterized by improved heat radiation, for advantageous use in an electron discharge device.

3. A metal element comprising a structure having thereon a coating of carbon for improved heat dissipation and being adapted to be worked and formed for use in an electron discharge device without appreciable loss of said coating, said structure comprising a non-porous base made of a metal selected from the group consisting of mild steel and nickel, and a nickel matrix bonding layer bonded to said base, said bonding layer consisting entirely of nickel particles individually having pores therein and sintered to each other, said bonding layer having an outer surface consisting of some of said particles, said some of said particles having voids therebetween and pores therein communicating with said surface, said coating filling said voids and pores, whereby said element has a continuous carbon coating characterized by increased heat dissipation and is adapted to be worked and formed with reduced loss of coating material.

30.

References Cited in the file of this patent

UNITED STATES PATENTS

|           |            |                |
|-----------|------------|----------------|
| 1,197,694 | Watkins    | Sept. 12, 1916 |
| 1,703,177 | Short      | Feb. 26, 1929  |
| 1,922,254 | McCullough | Aug. 15, 1933  |
| 2,133,761 | Tietig     | Oct. 18, 1938  |
| 2,147,447 | Kolligs    | Feb. 14, 1939  |
| 2,187,086 | Koehring   | Jan. 16, 1940  |
| 2,190,237 | Koehring   | Feb. 13, 1940  |
| 2,239,414 | Eddison    | Apr. 22, 1941  |
| 2,289,614 | Wesley     | July 14, 1942  |

FOREIGN PATENTS

|    |         |        |                |
|----|---------|--------|----------------|
| 45 | 965,421 | France | Sept. 12, 1950 |
|----|---------|--------|----------------|